

# UNITED STATES PATENT OFFICE.

LAWRENCE E. BARRINGER, OF SCHENECTADY, NEW YORK, ASSIGNOR TO GENERAL ELECTRIC COMPANY, A CORPORATION OF NEW YORK.

## INSULATING COMPOSITION.

1,091,725.

No Drawing.

Specification of Letters Patent. Patented Mar. 31, 1914.

Application filed January 18, 1913. Serial No. 742,971.

To all whom it may concern:

Be it known that I, LAWRENCE E. BARRINGER, a citizen of the United States, residing at Schenectady, county of Schenectady, State of New York, have invented certain new and useful Improvements in Insulating Compositions, of which the following is a specification.

The present invention comprises a composition suitable particularly for insulating electrical apparatus, such as transformers or generators and the like. Insulation of this character must not only be cheap, permanent, have high dielectric properties and be insoluble in the mineral oils used for cooling electrical apparatus, but must also have physical properties enabling it to be readily applied and retained by the coils or other objects to be impregnated. For example, it should be solid at operating temperatures, but fusible at a temperature attainable for impregnating the apparatus. Some fusible insulating compounds are more or less soluble in oils or have too high a flow point; others have a flow point which becomes progressively higher in the impregnating tank and finally the bath becomes unfit for further use by becoming too viscous.

I have found a mixture comprising gum copal, castor oil and the resin extracted by solvents from crude rubber, and known as "rubber resin" to meet all the above requirements.

Although a mixture of gum copal and castor oil has insulating properties and is insoluble in mineral oil, the flow point of the mixture of these substances when heated to about 150 deg. C. soon begins to ascend very rapidly, and within a very few days the mixture turns into a rubbery mass which cannot be liquefied by heating. In this condition the mixture, of course, is unfitted for the purpose of impregnation. When rubber resin is added to gum copal and castor oil, the composition will remain liquid at 150 deg. C. for two or three weeks or even longer. The flow point rises somewhat, but not to such

an extent as to cause the difficulty pointed out above. This mixture is, therefore, especially suitable for use in impregnating tanks where continuous liquidity is desirable to impregnate electrical coils, or the like.

I prefer to use a mixture in the following proportions:

|              |          |
|--------------|----------|
| Rubber resin | 8 parts. |
| Castor oil   | 10 "     |
| Gum copal    | 82 "     |

These proportions need not be strictly adhered to, but when the proportion of castor oil is varied, it changes the initial flow point of the material. When the proportion of castor oil is decreased the flow point will gradually rise and conversely the increase of castor oil content will lower the flow point. When it is desired that the initial flow point be above 100 deg. C., the castor oil should not be less than 5% and not over 15%. The proportion of rubber resin may be varied from about 5% to 20% and the proportion of gum copal from about 70 to 85%, depending somewhat on the proportion of the other ingredients. The mixture is insoluble in mineral oils, such as "transil oil," is very adhesive and has very high insulating properties.

In some cases the rubber resin may be replaced in part by ordinary resin, or colophony, with a consequent cheapening of the composition, but I find that when rubber resin alone is used as a flux the compound adheres better to the fabric insulation of the coils.

What I claim as new and desire to secure by Letters Patent of the United States, is:

1. A composition of matter comprising copal, castor oil, and rubber resin.
2. An insulating composition comprising by weight about 70 to 85 parts of copal, 5 to 15 parts of castor oil, and 5 to 20 parts of rubber resin.
3. A filler for oil immersed electrical coils comprising substantially by weight 82 parts gum copal, 10 parts, castor oil, and 8 parts

of resin extracted from crude rubber, characterized by high insulating properties, continued liquidity when heated and insolubility in mineral oil.

5. 4. An insulating composition consisting of gum copal, castor oil, rubber resin and colophony.

In witness whereof, I have hereunto set my hand this 17th day of January, 1913.

LAWRENCE E. BARRINGER.

Witnesses:

BENJAMIN B. HULL,  
HELEN ORFORD.